# EUROPEAN PATENT SPECIFICATION

(11) **EP 1 552 046 B1**
(45) Date of publication and mention of the grant of the patent: **08.08.2007**
(21) Application number: 02722457.5
(22) Date of filing: 30.04.2002
(51) Int. Cl.: D03D 1/00

(54) **LOOP PILE FABRIC**
POLSCHLINGENGEWEBE
TISSU A VELOURS BOUCLE

(30) Priority: 30.04.2001 GB 0110487
(43) Date of publication of application: 13.07.2005
(73) Proprietor: Christy UK Limited, Hyde, Cheshire SK13 4NR (GB)
(72) Inventor: ECCLES, David, c/o Christy UK Limited, Hyde, Cheshire SK14 4NR (GB); FINNEN, Rodney David, c/o Christy UK Limited, Hyde, Cheshire SK14 4NR (GB)
(74) Representative: Marshall, Caroline
(86) International application number: PCT/GB2002/001943
(87) International publication number: WO 2002/088442

(56) References cited:
- DE-A- 2 507 054
- GB-A- 345 432
- GB-A- 1 030 147
- US-A- 4 512 049

## Description

The present invention relates to a pile towelling fabric and products made from the towelling fabric.

Pile towelling fabrics are well known; they comprise a ground fabric which is covered on one or both of its faces with a projecting loop pile. The fabrics are normally woven and the pile forming yam is normally a warp yarn.

The main function of a towelling fabric is to dry the skin of a user by rubbing the towelling fabric over the skin. This main function of a towelling fabric is referred to herein as the 'towelling function'. The performance of the towelling function is primarily dependent upon two criteria; viz. the capability of the towelling fabric to physically remove droplets of water from the skin and the ability of the fabric to absorb the water which has been removed. Thus the greater the capability of being able to physically remove water droplets from the skin and the greater the capability to absorb water, then the higher the performance of the towelling function.

The capability of a towelling fabric to physically remove water droplets from the skin is dependent upon the degree to which the pile loops are upstanding and also the smoothness of the loop pile. In this respect, more upstanding loops are the better for 'grabbing' water droplets during rubbing of the towelling fabric over the skin. Also with regard to smoothness, the less smooth or slippy the pile loop the better. For instance, if the pile loops are too slippy, there is a tendency for the towelling fabric, when folded upon itself, to slide over itself rather than slide across the skin when a user attempts to rub the fabric over their skin. Thus if the loop pile is too slippy it detracts from the towelling function of the fabric.

A commonly used material for towelling fabrics is cotton. This is because cotton is sufficiently stiff to provide upstanding pile loops which are not too slippy and thereby provides a good capability for physically removing water droplets from the skin. In addition, cotton has good water absorbency characteristics. Thus, overall, a towelling fabric made from 100% cotton has a good towelling function.

It has been recognised by the present applicants that a certain market sector of users require a towelling fabric which has certain luxuriant qualities which render it highly desirable whilst having an underlying good absorbency function.

This market sector associates a natural silk content as rendering the towelling fabric as highly desirable. The greater the natural silk content, the greater the desirability.

The presence of a natural silk content in the towelling fabric is perceived by this market sector as providing the towelling fabric with certain qualities hereinafter referred to as 'desirability qualities'.

Unfortunately, natural silk is not well suited for incorporation into a towelling fabric since, primarily due to its slippy nature, it detracts from the towelling function of the fabric. Thus, although the presence of a high natural silk content may contribute to the desirability quality of the towelling fabric, the higher the natural silk content the poorer the towelling function of the towelling fabric.

Also, the present applicants have recognised that the market sector referred to above associate a high lustrous appearance to be an indication of the amount of natural silk contained in the fabric. Thus an important desirability quality is the lustrous visual appearance of the towelling fabric, i.e. the degree of shine and shimmer of the fabric. The present applicants have recognised that for a towelling fabric, a dull appearance (as commonly associated with towelling fabrics made from 100% cotton) detracts from the desirability quality of the fabric.

A general aim of the present invention is to provide a pile towelling fabric which incorporates a sufficiently high content of natural silk to give it a high desirability quality whilst retaining a good towelling function.

According to the present invention there is provided a pile towelling fabric having a ground fabric structure from which a pile projects, the pile being formed from a yam spun from a blend of staple fibres consisting of a combination of a first blend constituent comprising a moisture absorbent binding fibre and a second blend constituent including natural silk fibres.

The binding fibre is preferably highly moisture absorbent and preferably comprises cotton. Any variety of cotton may be used.

Preferably the second blend constituent comprises natural silk only or a combination of natural silk fibres and fibres of a soft, lustrous material such as a regenerated cellulose, eg modal, the lustrous fibres preferably having a greater degree of lustre than natural silk.

The natural silk content in the spun yam preferably ranges between 1 to 50% by weight, more preferably between 5 to 30% by weight, and still more preferably 10 to 25 % by weight of the spun yarn.

The presence of natural silk fibres in the second blend constituent of the spun yam provides the towel fabric with a lustrous silky appearance, a 'clingy' or fluid drape, and/or additional moisture absorbency.

The presence of the lustrous fibres in the second blend constituent provides additional moisture absorbency for the spun yam and contributes to the soft feel of the pile and the fluid drape of the fabric.

Preferably the regenerated cellulose fibre yarn is modal but other regenerated cellulose fibres such as Lyocell may be used. The modal may be micro modal having a dtex value of 1.0 or less; or alternatively may be a non-micro modal having a dtex value of about 1.5 dtex. Preferably the modal has a dtex value of 2 dtex or less. Micromodal is preferred as it increases the soft feel and improves the wicking capability of the pile yarn.

The lustrous fibre content is preferably between 20% to 40% by weight of the spun yarn; more preferably between 25 to 35% by weight of the spun yarn.

Preferably the second blend constituent constitutes 50% or more by weight of the spun yarn.

Preferably the percentage by weight of the first blend constituent in the spun yam is chosen to ensure that sufficient binding fibres are present to anchor the natural silk fibres, and if provided, the lustrous fibres of the second blend constituent within the spun yarn.

In this respect the natural silk and lustrous fibres of the second blend constituent tend to be smooth and prone to shed from the spun yarn. The first blend constituent is preferably composed of fibres which readily interlock during spinning, i.e. the fibres extend in a twisted manner and/or are hairy. These fibres therefore tend to positively lock or bind to one another.

In the spun blended yam of the present invention, the fibres of the first blend constituent interlock with the smooth natural silk and, if provided, the lustrous fibres of the second blend constituent and the quantity of the first blend constituent relative to the second blend constituent is chosen to be sufficiently great to ensure that the fibres of the second blend constituent are bound within the spun yarn.

Also the percentage weight of the first constituent in the spun pile yam is preferably chosen to ensure that pile loops formed from the pile yam are upstanding.

Preferably the pile is defined by pile loops. The loops preferably have a length which ranges between 10 to 20 mm, more preferably between 12 to 18 mm.

The ground fabric structure is preferably formed from a highly moisture absorbent yam such as cotton in order to improve the overall moisture absorbent capability of the towel. It has been found that the spun yam of the present invention exhibits good wicking capabilities and so ensures that moisture is transmitted to the ground fabric to be absorbed there.

Preferably the yam count of the cotton used for forming the ground structure is chosen to be sufficiently fine so as not to cause the towelling fabric to stiffen to mask the drape qualities imparted by the looped pile.

Preferably the yarn count of cotton yarn used for forming the ground fabric is about 12 ne.

Preferably the yam count of the spun pile forming yarn is about 16 ne.

Preferably the fabric is a woven fabric.

The blended yam is preferably combed prior to spinning in order to give a softer, more lustrous yarn which also is less prone to short fibre shedding.

Specific examples of a pile fabric according to the present invention are given below:-

| | | | | | |
|---|---|---|---|---|---|
| Fabric Type: | 3 pick terry weave | | | | |
| Blended Pile Yam: | Comb blend consisting of 48% by wt cotton/30% by wt micromodal and 22% by wt silk; yam count of 16 ne | | | | |
| Ground Warp: | Carded cotton; yarn count of 12 ne | | | | |
| Body Weft: | Open end spun cotton; yarn count of 12ne. | | | | |
| Size (cms): | 33 x 33 | 50 x 76 | 50 x 100 | 75 x 137 | 90 x 178 |
| Weight/Unit (g): | 65.4 | 243 | 330 | 678 | 1024 |
| Weight/M² (g): | 600 | 640 | 660 | 660 | 640 |
| Ends/cm: | 26.9 | 27.2 | 27.2 | 27.2 | 26.9 |
| Reed: | 58 | 58 | 58 | 58 | 58 |
| Picks/cm: | 16.9 | 18.5 | 19.3 | 19.7 | 19.3 |
| Terry Ratio: | 8.15 | 9.95 | 10.4 | 10.6 | 10.4 |
| Loop Length (mm): | 14.4 | 16.1 | 16.2 | 16.2 | 16.2 |

In the above examples, the cotton constituent in the spun pile yam provides moisture absorbency and binding of the modal and natural silk within the pile yarn. The modal constituent provides an increased rate of moisture absorbency due to its wicking capabilities, a soft feel and lustrous appearance. The silk constituent primarily provides durability, lustrous appearance and more fluid drape.

The pile yam of the above example exhibits good wickability to transfer moisture to the ground fabric whereat moisture is also absorbed. Thus, overall, the entire towelling fabric (i.e. the ground fabric and pile loops) exhibits good water absorbency.

It has also been surprisingly found that in the above example the 'towelling handle' of the towelling fabric, i.e. the tactile nature of the towelling fabric when a user touches or rubs the pile surface, is improved over that of the towelling handle characteristics of the individual constituents. This is perceived by the user to reflect the presence of natural silk within the fabric and so markedly improve its desirability quality.

In this respect, the towelling handle of a pile towelling fabric having pile made from 100% cotton has a soft feel due to the bulky nature of cotton but tends to feel harsh when rubbed due to the cotton defining relatively hard/stiff upstanding pile loops.

A towelling fabric having pile made from 100% natural silk fibres has a hard feel due to the lack of bulk provided by natural silk fibres and tends to feel slippy and damp when rubbed. The pile loops are upstanding ( to a lesser degree than with cotton) and due to the rigid/stiff nature of natural silk fibres the individual pile loops can be felt (likened to rubbing fingers along bristles).

A towelling fabric made from 100% modal also feels hard due to the lack of bulk and again feels slippy and damp when rubbed. The pile loops also lie flat and so also contribute to a hard feel when the pile is rubbed.

By contrast, a pile towelling fabric formed from a blended spun yam having 48% by weight cotton, 22% by weight natural silk fibres and 30% by weight modal, exhibits excellent towelling handle in that the pile yam produces a pile having upstanding loops and a bulked pile which is soft to the touch and also has a soft feel when rubbed.

It is to be appreciated that a reduction or increase in the relative proportions of the cotton, natural silk and modal fibres in the first and second constituents in the yam will have differing effects on the towelling function of the towelling fabric, its visual appearance and its towelling handle.

Thus a pile yam according to the present invention may have a relatively low natural silk and modal content but still provide a towelling fabric having superior desirability qualities (than a towelling fabric made of say 100% cotton) by improving the towelling handle and visual appearance of the towelling fabric.

For instance, such a towelling fabric may be provided by forming the pile loops from a spun yam having about 80% by weight of cotton, 10% by weight of natural silk and 10% by weight of modal.

As indicated above, the provision of the lustrous fibres in the second constituent improves the visual appearance of the towelling fabric in that it gives the fabric a higher degree of lustre than that possible with cotton and natural silk only and in addition provides a softer feel to the blended yarn than that felt when the spun yam comprises cotton and natural silk only.

However, it is envisaged that, although preferred, the presence of the lustrous fibres in the second constituent is optional. In this respect, a pile yam spun from a blend of cotton and natural silk fibres still provides improved towelling handle and improved visual appearance than when compared to a pile yam formed from either cotton or natural silk alone. In this respect it is envisaged that to achieve the benefits of towelling handle and visual appearance, the natural silk content may range between 1 to 50% by weight of the yam whilst the remainder of the yam is made up of cotton.

The pile towelling fabric of the present invention is particularly useful for making into towels of any size and for being made into garments such as bathrobes.

## Claims

1. A pile towelling fabric having a ground structure from which a pile projects, the pile being formed from a yarn spun from a blend of staple fibres consisting of a combination of a first blend constituent comprising a moisture absorbent binding fibre and a second blend constituent including natural silk fibres.

2. A pile fabric according to Claim 1 wherein the binding fibre comprises cotton.

3. A pile fabric according to Claim 1 or 2 wherein the second blend constituent constitutes 50% or more by weight of the spun yarn.

4. A pile fabric according to Claim 1, 2 or 3 wherein the second blend constituent comprises a combination of natural silk and fibres of a lustrous material.

5. A pile fabric according to Claim 4 wherein the lustrous fibres are made from a regenerated cellulose.

6. A pile fabric according to Claim 4 or 5 when dependent on claim 1 or 2 wherein the natural silk fibres constitute 1-50% by weight of the spun yarn.

7. A pile fabric according to Claim 6 wherein the natural silk fibres constitute about 22% by weight of the spun yarn.

8. A pile fabric according to Claim 4, 5, 6 or 7, wherein the lustrous fibres constitute between 20-50% by weight of the spun yarn.

9. A pile fabric according to Claim 5 or any of Claims 6 to 8 when dependent on Claim 5, wherein the lustrous fibres comprise modal fibres.

10. A pile fabric according to Claim 9 wherein the modal fibres have a dtex value of less than about 2 dtex.

11. A pile fabric according to any preceding claim wherein the blend of staple fibres are combed prior to spinning.

12. A pile fabric according to any preceding claims wherein the fabric is of a three pick terry weave construction.

## Patentansprüche

1. Ein Flor-Handtuchgewebe mit einer Grundstruktur, von der ein Flor absteht, wobei der Flor aus einem Garn gebildet ist, das aus einer Mischung von Stapelfasern gesponnen ist, die aus einer Kombination eines ersten Mischungs-Bestandteils umfassend eine feuchtigkeitsabsorbierende Bindungsfaser und eines zweiten Mischungs-Bestandteil enthaltend Naturseidenfasern besteht.

2. Ein Florgewebe gemäß Anspruch 1, wobei die Bindungsfaser Baumwolle umfaßt.

3. Ein Florgewebe gemäß Anspruch 1 oder 2, wobei der zweite Mischungs-Bestandteil 50 % oder mehr bezogen auf das Gewicht des gesponnenen Garns bildet.

4. Ein Florgewebe gemäß Anspruch 1, 2 oder 3, wobei der zweite Mischungs-Bestandteil eine Kombination aus Naturseide und Fasern eines glänzenden bzw. schimmernden Materials umfaßt.

5. Ein Florgewebe gemäß Anspruch 4, wobei die glänzenden bzw. schimmernden Fasern aus einer regenerierten Zellulose hergestellt sind.

6. Ein Florgewebe gemäß Anspruch 4 oder 5 in Abhängigkeit von Anspruch 1 oder 2, wobei die Naturseidenfasern 1-50% bezogen auf das Gewicht des gesponnenen Garns bilden.

7. Ein Florgewebe gemäß Anspruch 6, wobei die Naturseidenfasern etwa 22% bezogen auf das Gewicht des gesponnenen Garns bilden.

8. Ein Florgewebe gemäß Anspruch 4, 5, 6 oder 7, wobei die glänzenden bzw. schimmernden Fasern zwischen 20-50% bezogen auf das Gewicht des gesponnenen Garns bilden.

9. Ein Florgewebe gemäß Anspruch 5 oder einem der Ansprüche 6 bis 8 in Abhängigkeit von Anspruch 5, wobei die glänzenden bzw. schimmernden Fasern Modalfasern umfassen.

10. Ein Florgewebe gemäß Anspruch 9, wobei die Modalfasern einen dtex-Wert von weniger als etwa 2 dtex haben.

11. Ein Florgewebe gemäß einem voranstehenden Anspruch, wobei die Mischung aus Stapelfasern vor dem Spinnen gekämmt werden.

12. Ein Florgewebe gemäß einem der voranstehenden Ansprüche, wobei das Gewebe einen Frottee-Bindungsaufbau mit drei Schussschlägen besitzt ("three pick terry weave construction").

## Revendications

1. Tissu en tissu éponge à poils ayant une structure de base à partir de laquelle un poil fait saillie, le poil étant formé à partir d'un fil filé à partir d'un mélange de fibres courtes constituées d'une combinaison d'un premier constituant de mélange comprenant une fibre liante absorbant l'humidité et d'un second constituant de mélange comprenant des fibres en soie naturelle.

2. Tissu à poils selon la revendication 1, dans lequel la fibre liante comprend du coton.

3. Tissu à poils selon la revendication 1 ou 2, dans lequel le second constituant de mélange constitue 50 % ou plus en poids du fil filé.

4. Tissu à poils selon la revendication 1, 2 ou 3, dans lequel le second constituant de mélange comprend une combinaison de soie naturelle et de fibres d'un matériau brillant.

5. Tissu à poils selon la revendication 4, dans lequel les fibres brillantes sont constituées d'une cellulose régénérée.

6. Tissu à poils selon la revendication 4 ou 5 lorsqu'elle dépend de la revendication 1 ou 2, dans lequel les fibres en soie naturelle constituent 1 à 50 % en poids du fil filé.

7. Tissu à poils selon la revendication 6, dans lequel les fibres en soie naturelle constituent environ 22 % en poids du fil filé.

8. Tissu à poils selon la revendication 4, 5, 6 ou 7, dans lequel les fibres brillantes constituent entre 20 et 50 % en poids du fil filé.

9. Tissu à poils selon la revendication 5 ou selon l'une quelconque des revendications 6 à 8 lorsqu'elle dépend de la revendication 5, dans lequel les fibres brillantes comprennent des fibres en modal.

10. Tissu à poils selon la revendication 9, dans lequel les fibres en modal ont une valeur dtex inférieure à environ 2 dtex.

11. Tissu à poils selon l'une quelconque des revendications précédentes, dans lequel le mélange de fibres courtes est peigné avant le filage.

12. Tissu à poils selon l'une quelconque des revendications précédentes, dans lequel le tissu est d'une construction d'armure pour tissu éponge à trois duites.
